

Nov. 24, 1931.

H. F. FRUTH

1,833,641

MICROPHONIC MATERIAL AND METHOD OF PRODUCING THE SAME

Filed March 15, 1930

Fig. 1



Fig. 2.



Fig. 3.



Inventor  
H. F. FRUTH

By J. H. B. Whitfield Atty.

## UNITED STATES PATENT OFFICE

HAL F. FRUTH, OF RIVERSIDE, ILLINOIS, ASSIGNOR TO WESTERN ELECTRIC COMPANY,  
INCORPORATED, OF NEW YORK, N. Y., A CORPORATION OF NEW YORK

## MICROPHONIC MATERIAL AND METHOD OF PRODUCING THE SAME

Application filed March 15, 1930. Serial No. 436,175.

This invention relates to microphonic material and methods of producing the same, and more particularly to a material consisting of particles of insulating substance 5 coated with a conducting layer, for use in microphones, telephone transmitters and repeaters, and like instruments, and to methods of producing such material.

Objects of the invention are to provide 10 an improved microphonic material and method of producing the same; to provide a microphonic material of superior elasticity and sensitivity; and to provide a microphonic material of relatively low specific gravity.

15 In general terms, the present invention contemplates the use as a microphonic material of particles of an elastic substance such as glass or other vitreous substance, each particle being coated with a thin layer of 20 metal, such as platinum or iridium, or other conducting substance. In order to decrease the specific gravity of the material to the point where it will compare favorably with the carbon granules commonly used as a 25 microphonic material, the insulating substance has incorporated therein bubbles of air or other gas, which may be formed by suitably working the insulating substance while in molten form or may be formed by 30 mixing a gas-generating substance in the molten insulating substance to form the bubbles autogenously. The invention further contemplates an improved method for producing a layer of conducting substance upon the 35 surface of the insulating substance. Such layer may be formed by incorporating the conducting substance in the insulating substance, forming the resulting material into particles, and subsequently reducing the material by any suitable treatment to leave a 40 residue of conducting substance on the surfaces of the particles. The particles used as microphonic material are preferably of spherical or spheroidal shape, although granular particles may also be used.

The invention will be more fully understood from the following description, taken in connection with the appended drawings, in which

50 Fig. 1 is an enlarged cross-sectional view

showing the insulating material having gas bubbles incorporated therein,

Fig. 2 is an enlarged sectional view of a spherical particle having a coating of conducting substance thereon, and

Fig. 3 is an enlarged sectional view of a granule of the same material having a coating of conducting substance thereon.

In the drawings, which are to be construed as illustrating the invention rather than 60 limiting it, the reference numeral 10 designates generally a piece of glass or other fusible insulating substance having incorporated therein bubbles 11 of air or other gas. These bubbles may be formed by mixing with 65 the insulating substance a substance which, upon being raised to a temperature above the melting point of the insulating substance, will generate gas in quantities sufficient to form the bubbles. In practicing such a process, the insulating substance and the gas generating substance may be mixed together in 70 granular or powdered form and the mixture is then raised to the melting point of the insulating substance and to such higher temperature as may be necessary to cause the 75 generation of gas, whereupon the material is cooled and reduced to particles of suitable size as described below.

Another method of forming the article 80 illustrated in Fig. 1 is to agitate molten glass in such a manner as to cause it to become "seedy"; that is, filled with bubbles. This may be done by alternately drawing out and folding upon itself a small portion of molten 85 glass, causing bubbles to become incorporated therein in the manner known to those skilled in the art, or it may be accomplished by other agitating methods known in the art. The material may then be comminuted 90 and solidified in a shot tower in the known manner, forming globules as indicated in Fig. 2, or it may be chilled and crushed to reduce it to small particles of granular shape 95 as indicated in Fig. 3. These particles may then be sifted to select the granules of the proper size, granules which pass a 50-mesh screen and are retained on a 100-mesh screen being suitable for most purposes, although the size of the particles may be widely va- 100

ried depending upon the particular nature of the instrument in which the material is to be used, and upon other factors.

The coating of metal or other conducting substance 12 may be applied to the particles by cathodic sputtering in the manner disclosed in my copending application Serial No. 329,645, filed December 31, 1928, or it may be applied in any other suitable known manner. One satisfactory manner of applying the coating is by incorporating in the molten material a salt of the metal, such as gold chloride, dissolving the salt in the molten vitreous material, then forming the mixture into globules or granules, and subsequently reducing the salt at the surface of the globules or granules by subjecting them to a reducing atmosphere at a high temperature. The metallic salt may also be dissolved in a glaze, which may then be applied to the globules or granules as a coating and subsequently subjected to a reducing process. Either of these treatments leaves a metallic deposit upon the globules which is uniform and satisfactory for microphonic purposes. The coating 12 may also be applied by applying to the particles a liquid solution of a compound of the metal, and then precipitating the metal therefrom upon the surfaces of the particles, the process being similar to that employed in the silvering of mirrors. It is also possible to coat the particles by vaporizing the metal or a compound thereof and condensing the vapor upon the surfaces of the particles in a manner similar to the well known sherardizing process. Various mechanical methods may also be employed, such as tumbling the particles in contact with the metal to be applied thereto, or applying the metal in the form of a paint and subsequently burning out the combustible ingredients of the paint to leave a residue of conducting metal.

The microphonic material described herein may be manufactured at a relatively low cost, and is very elastic and durable in use.

While the invention has been described specifically, it is to be understood that various changes may be made without departing from the spirit of the invention as defined in the following claims.

What is claimed is:

1. Microphonic material consisting of metal-coated glass beads having gas bubbles incorporated therein.

2. Microphonic material consisting of particles of glass having air bubbles incorporated therein, and coated with a noble metal.

3. A method of producing microphonic material which consists in forming air bubbles in glass, forming the glass into particles of substantially uniform size, and coating the particles with metal.

4. A method of producing microphonic material which consists in working molten

glass to produce air bubbles therein, forming the glass into particles, and coating the particles with metal.

5. A method of producing microphonic material which consists in working molten glass to produce air bubbles therein, solidifying and reducing the glass to small particles, selecting particles of a substantially uniform size and coating the selected particles with a conducting material.

6. A method of producing microphonic material which consists in incorporating into a vitreous material a compound of an insulating material, forming the mixture into particles, and reducing the compound at the surfaces of the particles to leave a coating of conducting material thereon.

7. Microphonic material consisting of platinum-coated particles of glass having gas bubbles incorporated therein.

8. Microphonic material consisting of spheroidal particles of glass coated with a noble metal and having gas bubbles incorporated therein.

9. Microphonic material consisting of particles of glass having air bubbles incorporated therein and coated with a noble metal by a cathodic sputtering process.

In witness whereof, I hereunto subscribe my name this 28th day of February, A. D. 1930.

HAL F. FRUTH.

100

105

115

120

125

130